

1

3,328,117

**PROCESS FOR PRODUCING FIBROUS ALKALI METAL TITANATES**

Robert S. Emslie, Chadds Ford, Pa., and Hugh C. Gullidge, Newark, and George L. Lewis and Oswin Burr Willcox, Wilmington, Del., assignors to E. I. du Pont de Nemours and Company, Wilmington, Del., a corporation of Delaware  
No Drawing. Filed May 10, 1963, Ser. No. 279,580  
23 Claims. (Cl. 23—51)

This invention relates to improved fibrous alkali metal titanates and to novel methods for their preparation.

More particularly, it relates to selectively synthesizing improved, water-insoluble fibrous alkali titanates in various diameters and lengths and by means of a novel non-fluid reaction process in which observance of certain temperature controls and other conditions insures the selective production of such fibrous products in predominant desired colloidal, pigmentary or insulating size ranges.

U.S. Patent 2,833,620 discloses the preparation of fibrous dialkali metal titanates corresponding to the formula  $M_2O(TiO_2)_n$ , in which  $n$  is 6—7 and  $M$  is an alkali metal having an atomic number greater than 11, i.e. sodium, potassium, rubidium, and cesium by reacting in the presence of water a water-soluble basic oxygen-containing alkali metal compound, such as an alkali metal hydroxide, with an oxygen-containing titanium compound, such as titanium dioxide, at a temperature of at least 400° C. under a pressure of at least 200 atmospheres. U.S. 2,841,470 discloses the preparation of fiber of the general formula  $M_2O(TiO_2)_{2n}$  where  $n=2-3$  by dissolving a non-fibrous alkali metal titanate in a fused, heated salt melt of an alkali metal chloride or fluoride, maintaining a portion of the molten halide saturated with the dissolved compound as the fibrous alkali metal titanate is formed, and separating the crystallized titanate fibers from the salt by water extraction.

In accordance with this invention, selective production can be effected of an improved fibrous alkali metal titanate in either predominantly colloidal, pigmentary or insulating type, by recourse to novel process techniques which are readily adaptable for continuous commercial operation and from which recovery is obtained of relatively large, increased yields of fiber product per unit charged to the system. Advantageously, this is achieved without recourse to costly pressure equipment and procedures, or experiencing the difficult containment, heating and handling problems incidental to liquid molten salt mixture use.

These and other major advantages are attained in this invention which embodies the discovery that observance of a precise control over the temperatures of calcination within a range of from about 200° C. to 1150° C., and preferably from about 600—1100° C. in a continuous operation to react a non-fluid (substantially free from any liquid or gaseous phase) reaction mixture comprising a basic oxygen-containing alkali compound, such as an alkali metal hydroxide or carbonate, and an oxygen-containing titanium compound, such as titanium dioxide, in such proportions as will yield a fibrous titanate product containing a ratio of  $TiO_2/M_2O$  (wherein  $M$  is an alkali metal) ranging from 4:1 to 9:1 and preferably from 4:1 to 7:1, provides an effective control over the development and ultimate length and diameter of such product. In consequence, production will be assured of a titanate material of greatly improved uniformity, e.g. its fibers will be in the desired dimensions and free of substantial percentages of undersized and oversized material. Thus, when in accordance with the invention, relatively low, from about 200—850° C. and preferably from 600—825°

2

C. temperatures are resorted to, the fibrous material will be found to comprise particles predominantly (that is in excess of 50% and preferably at least 80% thereof) which are in colloidal dimension to range from .005—0.1 5 micron in diameter with lengths at least 10 times said diameter; when calcination temperatures in the range from about 850—975° C. are undertaken, a fibrous product predominantly in pigmentary size range will result, having a particle diameter ranging from 0.1—0.6 micron with 10 lengths ranging from 10 to 100 times the said diameter; and when temperatures ranging from about 975° C., to 1150° C., and preferably from about 975° C. to 1150° C. are utilized, one obtains a fibrous product of predominantly greater dimension having a particle diameter ranging 15 from 0.6—3.0 microns with length of from 100—1000 times the diameter and longer which possesses great utility as an insulating or reinforcing material. These size ranges of products can be readily determined by examination with an electron microscope at a magnification at 25,000 to 20 50,000 times actual size and measuring directly the enlarged image of the product.

In producing the improved fibrous alkali metal titanates of this invention, a dry, compacted intimate reaction mixture or charge is first prepared by suitably dry blending the various reactant components and then briquetting or otherwise conventionally converting the blend into lump or compacted form. The compacted charge can comprise a mixture of a basic oxygen-containing alkali metal compound, particularly a hydroxide or carbonate 25 of sodium or potassium, with a titanium compound, particularly titanium dioxide, with the latter preferably being in a suitably divided form for uniform dispersion throughout the mixture. The equivalent molar ratio of titanium compound to alkali metal compound, calculated as 30 titanium dioxide to alkali metal oxide ( $TiO_2/M_2O$  wherein  $M$  preferably consists of K or Na) is variable, and can range from 2:1 to 8:1. Preferably, such ratio ranges from 3:1 to 5:1. Alternatively, an alkali metal halide salt, particularly a chloride of potassium or sodium, can be 35 introduced as a component of the charge, and in amounts ranging from about 5—65% by weight based on the total weight of the charge. In such event, the amount of basic oxygen-containing alkali compound present can range from about 7—65% and the amount of titanium oxygen-containing compound used can range from about 20—45 80% by weight to provide a 0.25 to 20 mole ratio of  $TiO_2/M_2O$ .

The resulting compact is then converted to the desired colloidal, pigmentary or insulating form of fibrous titanate, 50 by calcining it in conventional furnacing means such as a direct-fired batch or rotary kiln or shaft type furnace and on a continuous basis. The calcination can be conducted over periods of time ranging from about 0.25 to 16 or more hours, depending upon the nature and composition 55 of the dry reaction charge, the type of fibrous titanate being produced, and the particular temperatures and furnacing means utilized. For example, in the calcination, the reaction charge can be continuously fed to the cooler temperature end of a direct-fired rotary kiln or shaft furnace which is suitably maintained within the required temperature range, and from which the converted reaction product is continuously withdrawn from the hotter end of the furnace.

The fibrous titanate-containing calciner discharge 60 covered is then purified and separated from undesired reaction or other products through water or acid leaching treatment. Fibers are further separated by exfoliation. Thereafter it can be dried or otherwise treated to recover the desired final form of fibrous material. This process of purification and exfoliation can be carried out simultaneously with other processes like papermaking where crude kiln discharge is added directly to the beater. De-

pending on the form or type of fibrous product obtained, the material will be found to be highly useful in all applications where its inertness and other physical characteristics (like refractive index, aspect ratio, surface nature, and others, etc.) are requisite. For example, when such product is in preponderantly colloidal form it provides to be highly useful as an adjuvant for incorporation into lubricants, such as silicone grease to improve lubricant properties at higher temperatures. Similarly, when the product is preponderantly in pigment size range, it will be found to be advantageously useful in pigmenting paper or in compositions used in coatings on paper and folding boxboard. In such applications it will be found to be of enhanced value due to its highly desirable properties of 10 opacity, retention, brightness and the like which are attributable to its fiber length, diameter and melting point.

We have found, for example, that in making a sheet of paper of approximately 50 pound ream weight (500-25" x 40" sheets, to the ream), with an ash content of 6%, only 75% as much pigmentary potassium titanate, by weight, is required to achieve the equivalent opacity or "dry hiding power" of the sheet as is produced by 100% of a standard grade of water dispersible, anatase titanium dioxide pigment. This unexpected result is the more remarkable inasmuch as the refractive index of potassium titanate is only about 2.3 while that of anatase titanium dioxide is 2.5 and would be expected to impart a higher opacity, rather than a lower one, to the pigmented paper composition.

Likewise production of a preponderantly fibrous in-

an 11" I.D. by 13" internal length ceramic-lined kiln, rotating at 2 r.p.m. and fired directly with a gas burner by injecting the flame into one end of the kiln. On completion of the calcination, the reaction product discharge from the kiln was leached until freed of unreacted material and the compressed briquetted fibers were then crushed to a 4 mesh size and dispersed for 5 to 10 minutes in 4 gallons of distilled water, employing a conventional high speed, high shear type blender in the process. The fibers were then exfoliated by first adjusting the dispersion to a pH of 10.5 with dilute acetic acid and then passing the slurry through a colloid mill about 4-5 times. This dispersion was then run through a basket type centrifuge provided with a nylon filter cloth backed with cotton, dried, and evaluated. In colloid fiber processing the filtrate was saved while the filter cake was reslurried with 2 gallons of water and passed through the colloid mill an additional 4 times. Filtration through the centrifuge was repeated on the second dispersion. Filtrates were combined and acidified to a pH of 6.5 by adding a commercial cationic ion exchange resin while stirring for a period of 30-40 minutes. The resin was separated from the mix by filtration through a 200 mesh sieve. To the filtrate was added a commercial anion exchange resin while stirring for 30-40 minutes. This resin was removed through sieving prior to flocculation of the particles by the addition of 15 gms of alum in a 4% aqueous solution. Flocculated material was collected in the basket centrifuge. Filter cakes were dried at 95° C. and weighed. A summary of the results and products obtained are shown in the following Table I.

TABLE I

|   | Ingredients              |                                 | Composition of Reactor Mix, Parts by Wt. |                  | Reaction Temp., °C. | Time at Temp., (Hrs.) | Conversion to Fiber of Size, Percent | TiO <sub>2</sub> /M <sub>2</sub> O | Diameter (Range), Microns | Length (Range), Microns | Size Category <sup>1</sup> |
|---|--------------------------|---------------------------------|------------------------------------------|------------------|---------------------|-----------------------|--------------------------------------|------------------------------------|---------------------------|-------------------------|----------------------------|
|   | TiO <sub>2</sub>         | M <sub>2</sub> O                | TiO <sub>2</sub>                         | M <sub>2</sub> O |                     |                       |                                      |                                    |                           |                         |                            |
| A | Titania                  | K <sub>2</sub> CO <sub>3</sub>  | 160                                      | 138              | 600                 | 4                     | 100                                  | 4.3                                | 0.01-0.1                  | 1-2                     | C                          |
| B | do                       | K <sub>2</sub> CO <sub>3</sub>  | 160                                      | 138              | 750                 | 4                     | 100                                  | 4.5                                | 0.01-0.1                  | 1-2                     | C                          |
| C | do                       | K <sub>2</sub> CO <sub>3</sub>  | 160                                      | 138              | 800                 | 4                     | 100                                  | 5.0                                | 0.01-0.1                  | 1-2                     | C                          |
| D | do                       | KOH                             | 280                                      | 112              | 600                 | 4                     | 98                                   | 4.6                                | 0.01-0.1                  | 1-2                     | C                          |
| E | do                       | KOH                             | 280                                      | 112              | 750                 | 4                     | 100                                  | 5.3                                | 0.01-0.1                  | 1-2                     | C                          |
| F | do                       | Na <sub>2</sub> CO <sub>3</sub> | 400                                      | 106              | 700                 | 5                     | 75                                   | 5.1                                | .01-0.1                   | 1-2                     | C                          |
| G | do                       | NaOH                            | 320                                      | 112              | 850                 | 2                     | 95                                   | 5.1                                | .01-4                     | .5-1.6                  | P                          |
| H | do                       | Na <sub>2</sub> CO <sub>3</sub> | 400                                      | 106              | 900                 | 5                     | 90                                   | 5.9                                | .25-0.6                   | 10-30                   | P                          |
| I | do                       | NaOH                            | 320                                      | 112              | 875                 | 3                     | 75                                   | 4.6                                | .25-4                     | 10-20                   | P                          |
| J | do                       | NaOH                            | 320                                      | 112              | 875                 | 4                     | 85                                   | 6.2                                | .25-4                     | 10-20                   | P                          |
| K | Hydrous TiO <sub>2</sub> | KOH                             | 320                                      | 112              | 800                 | 6                     | 90                                   | 8.1                                | .25-4                     | 10-20                   | P                          |
| L | TiO <sub>2</sub>         | NaOH/50%                        | 320                                      | 100              | 875                 | 6                     | 95                                   | 5.3                                | .3-6                      | 10-25                   | P                          |
| M | TiO <sub>2</sub>         | 50%KOH                          | 320                                      | 100              | 875                 | 6                     | 95                                   | 6.2                                | .3-6                      | 10-25                   | P                          |
| N | Hydrous TiO <sub>2</sub> | K <sub>2</sub> CO <sub>3</sub>  | 500                                      | 100              | 1,090               | 16                    | 36                                   | 5.8                                | .74-1.3                   | 100-1,000               | I                          |

<sup>1</sup> C = Colloidal; P = Pigmentary; I = Insulating.

sulating form of product will possess high utility as a re-inforcing agent in fibers or papers and as an insulation material. Pigmentary size fibers can be used to form insulating compositions also. However, the insulation size fibers are particularly well suited since they produce blocks and felts of higher strength and lower density.

To a clear understanding of the invention the following illustrative examples and tables are given wherein parts mentioned are by weight. These are merely illustrative and are not to be construed as limiting the underlying principles and scope of the invention.

#### Example I

The following series of colloidal, pigmentary and insulating forms of fibrous potassium or sodium hexatitanate preparation was undertaken by calcining various blends and ratios of the alkali metal and titanium compounds enumerated in Table I below. The TiO<sub>2</sub> and other reactant ingredients employed were first dry-blended in a drum roller and then briquetted to approximately 1/2" x 1" x 1" size through a conventional compacting device at a pressure of 3300 lbs./sq. in.

The briquetted products were then calcined at the temperatures and for the time periods specified in Table I in

colloidal potassium titanate fibers in accordance with the invention, are the following series of calcinations applied to briquettes prepared from a master blend of TiO<sub>2</sub>, K<sub>2</sub>CO<sub>3</sub>, and KCl. This blend was prepared by dry blending the ingredients in a drum roller in a weight ratio of 2 parts TiO<sub>2</sub>/1 part K<sub>2</sub>CO<sub>3</sub>/1 part KCl (50% TiO<sub>2</sub>, 25% K<sub>2</sub>CO<sub>3</sub> and 25% KCl) where the TiO<sub>2</sub>/K<sub>2</sub>O mole ratio is 3.5/1. Briquettes of approximately 1/2" x 1" x 1" dimension were prepared from this dry blend by compaction at a pressure of 3300 lbs. per sq. in.

Three pounds of these briquettes were calcined in an 11" I.D. x 13" internal ceramic-lined kiln rotating at 2 r.p.m. and fired directly with a gas burner by injecting its flame into one end. Time at a temperature for various runs are shown in Table II below.

After calcination the calciner discharge was leached and purified as well as exfoliated as in Example I to provide the desired fibrous potassium titanate.

#### Example II

TABLE II

|   | Calcination Temp., °C. | Calcination Time, Hrs. | Percent Yield of Colloidal Size |
|---|------------------------|------------------------|---------------------------------|
| A | 775                    | 0.5                    | 7                               |
| B | 775                    | 0.5                    | 9                               |
| C | 775                    | 2.0                    | 11                              |
| D | 800                    | 0.5                    | 39                              |
| E | 800                    | 1.0                    | 63.5                            |
| F | 800                    | 2.0                    | 65                              |
| G | 800                    | 2.5                    | 52                              |
| H | 800                    | 3.0                    | 33                              |
| I | 815                    | 0.5                    | 48                              |
| J | 815                    | 1.0                    | 70                              |
| K | 815                    | 1.5                    | 79                              |
| L | 815                    | 2.0                    | 71                              |
| M | 815                    | 3.0                    | 42                              |
| N | 825                    | 0.5                    | 33                              |
| O | 825                    | 1.5                    | 57                              |
| P | 825                    | 2.0                    | 50                              |

Samples of this colloidal size fibrous potassium titanate product were incorporated into silicone grease with desired improvement and enhancement resulting in lubricating properties at relatively high temperatures.

*Example III*

A mixture containing 1 part of potassium carbonate, 2 parts of anatase titanium dioxide pigment and 1 part of potassium chloride was dry blended in a drum roller. The mole ratio of  $TiO_2:K_2O$  was 3.5 in the presence of 25 wt. percent potassium chloride. This material was then pressed into cylindrical briquettes of approximately  $\frac{3}{4}''$  x 1" size, which were then continuously fed, at rates varying from 20-75 lbs. per hour, into a gas-fired rotary ceramic-lined kiln with an 18" internal diameter and 30 ft. in length, heated by direct gas firing at the opposite end. The bed temperature within the kiln was adjusted to temperatures ranging from 600° at the feed port to 1200° C. at the exit, with a continuous increase in temperature existing over the 30 ft. length. Residence time of the reactants in the kiln was regulated at  $\frac{1}{2}$  to 6 hours being maintained by adjusting the pitch and rotary speed of the kiln. A uniform bed depth was maintained within the kiln, with the holdup amounting to anywhere between 150 lbs. to 450 lbs. of feed material for each run listed in the series shown in Table III below. A total of 2000 lbs. of briquettes containing the fibrous material were collected at the hot end of the kiln over each run period.

The time and temperature, the percent conversion to fibrous material of the size range listed, and the analysis of the water extracted product, as well as the size category in which the product obtained fell are shown in said Table III.

The calcined briquettes containing the fibrous material from each run were charged to 1000 gal. tanks and purged at 90° C. with demineralized water, timed at 3 gals. per hour for six days in the case where pigmentary and insulation grade fibers were formed (runs F through A-1). Colloidal fibrous material (runs A through E) were treated in a manner similar to that described in Example II. The leached fibers in bundles the shape of the briquettes originally fed to the kiln, were dried on trays in an oven at 110° C.

In the instance of pigmentary sized fibers, exfoliation was performed by first dry grinding the dry material through a four mesh screen, then mixing with demineralized water to form a 10% fiber slurry. This slurry was then passed through an attrition mill set at 3 mils and the slurry diluted to 1½% fiber content with additional demineralized water and passing this mixture through a cleaner consisting essentially of a wet cyclone separator to remove large particles of grit. Finally, the degritted slurry was reprocessed back through the attrition mill. The resulting dispersion was then pumped into a 3000 gal. vessel and allowed to settle for two hours. The top 10% of the liquid containing dispersed fiber was decanted and transferred to another tank and processed in 300 gal. portions as follows: The dispersed fiber slurry was neutralized to a pH of approximately 7.25 with 25% hydrochloric acid and flocculated by adding 7 lbs. of potassium chloride. Flocculated fibers were filtered on paper to form cakes 26" x 26" x 1" and were washed free of chloride with 3 or 4 portions of water 9 gals. each. The filter cakes were placed on trays and dried at 75° C. for 24 hrs. Moisture in the cake after drying average 3-5%. Dry filter cakes were exfoliated again by dry grinding to pass a four mesh screen, then micro-pulverized using a Metals Disintegrators, Inc. machine. The fibrous potassium titanate products were then sampled, sized and analyzed to provide the results as shown in Table III.

The insulation sized fibers shown were not ground in the manner described for the pigmentary sized fibers, but were simply exfoliated by dry grinding and were then formed into mats or felts of loose fibers and processed.

TABLE III

|     | Temperature, °C. | Time (Hrs.) at Temp. | Conversion to Fibers of size | Analysis of Water Extracted Product |                           |                         | Size Category <sup>1</sup> |
|-----|------------------|----------------------|------------------------------|-------------------------------------|---------------------------|-------------------------|----------------------------|
|     |                  |                      |                              | Mole Ratio $TiO_2/M_2O$             | Diameter average, microns | Length average, microns |                            |
| A   | 800              | 0.5                  | 15                           | 4.1                                 | 0.007                     | 0.6                     | C                          |
| B   | 800              | 1.0                  | 60                           | 5.2                                 | 0.01                      | 1.5                     | C                          |
| C   | 800              | 2.5                  | 75                           | 4.8                                 | 0.02                      | 2.0                     | C                          |
| D   | 800              | 3.5                  | 83                           | 6.7                                 | 0.08                      | 3.0                     | C                          |
| F   | 875              | 3                    | 75                           | 4.5                                 | 0.2                       | 2                       | P                          |
| G   | 875              | 6                    | 95                           | 6.2                                 | .4                        | 10                      | P                          |
| H   | 900              | 1                    | 50                           | 6.3                                 | .2                        | 2                       | P                          |
| I   | 900              | 3                    | 90                           | 5.8                                 | .4                        | 8                       | P                          |
| J   | 900              | 6                    | 98                           | 5.9                                 | .5                        | 12                      | P                          |
| K   | 925              | 1                    | 75                           | 4.2                                 | .5                        | 10                      | P                          |
| L   | 925              | 3                    | 95                           | 5.4                                 | .5                        | 15                      | P                          |
| M   | 925              | 6                    | 98                           | 6.8                                 | .6                        | 20                      | P                          |
| N   | 950              | 1                    | 85                           | 7.3                                 | .6                        | 15                      | P                          |
| O   | 975              | 1                    | 90                           | 9.2                                 | 1                         | 50                      | I                          |
| P   | 975              | 3                    | 95                           | 6.7                                 | 1                         | 75                      | I                          |
| Q   | 975              | 6                    | 99                           | 5.8                                 | 1                         | 100                     | I                          |
| R   | 1,025            | 1                    | 85                           | 4.9                                 | 1.2                       | 75                      | I                          |
| S   | 1,025            | 3                    | 97                           | 5.7                                 | 1.3                       | 100                     | I                          |
| T   | 1,025            | 6                    | 99                           | 6.0                                 | 2                         | 150                     | I                          |
| U   | 1,050            | 0.75                 | 95                           | 5.6                                 | 2                         | -----                   | I                          |
| V   | 1,050            | 1                    | 95                           | 7.2                                 | 1.5                       | 100                     | I                          |
| W   | 1,050            | 3                    | 98                           | 8.3                                 | 2.0                       | 150                     | I                          |
| X   | 1,050            | 6                    | 99                           | 6.3                                 | 3.0                       | 140                     | I                          |
| Y   | 1,075            | 1                    | 96                           | 4.3                                 | 2.0                       | 140                     | I                          |
| Z   | 1,075            | 3                    | 98                           | 9.1                                 | 3.0                       | 150                     | I                          |
| A-1 | 1,075            | 6                    | 99                           | 6.4                                 | 3.0                       | 150                     | I                          |

<sup>1</sup> C=Colloidal; P=Pigmentary; I=Insulating.

## Example IV

In this example fibrous potassium titanate materials were prepared in the same manner and in the apparatus described in Example III but using as sources of titanium dioxide, raw hydrous titania, the product from a commercial sulfate process for producing anatase  $TiO_2$  pigment, highly refined anatase pigment, ground rutile ore and beneficiated ilmenite. These reactants were mixed and compacted with various sources and amounts of potassium oxide, in the form of potassium carbonate, potassium bicarbonate in varying portions of potassium fluoride and chloride salts as shown in Table IV below. The reaction temperatures listed are the average temperatures at the time given. The analysis of the water extracted product, size category and other results obtained are also listed in the table.

Sodium titanate fibers in colloidal, pigmentary and insulation size ranges were manufactured employing the procedures and apparatus described in Example III, using the reactants, ratios and temperature conditions listed in (a) of Table V below and with the results therein shown.

In addition, mixed sodium and potassium titanate fibers were prepared in the same manner, utilizing the listed reactants, proportions and temperatures set forth in (b) of Table V to obtain the results therein given. The pigmentary potassium mixed titanate fibers were exfoliated by means of colloid mill treatment and were passed through this mill in a 1% slurry until the grit content (large sized particles) averaged less than 2% by weight. The insulation sized materials were dispersed in distilled water and washed until chloride free. Examples of these

TABLE IV

|   | Ingredients      |                  |      | Composition of Reaction Mix, Parts by Wt. |                  |      | Reaction Temp., °C. | Time (hrs.) at Temp. | Conversion to Fibers of Size, Percent | Analysis of Water Extracted Product           |                  |                | Size Category <sup>1</sup> |
|---|------------------|------------------|------|-------------------------------------------|------------------|------|---------------------|----------------------|---------------------------------------|-----------------------------------------------|------------------|----------------|----------------------------|
|   | TiO <sub>2</sub> | M <sub>2</sub> O | Salt | TiO <sub>2</sub>                          | M <sub>2</sub> O | Salt |                     |                      |                                       | Mole Ratio TiO <sub>2</sub> /M <sub>2</sub> O | Diameter (range) | Length (range) |                            |
| A |                  |                  |      | 62                                        | 33               | 5    | 930                 | 2.5                  | 95                                    | 5.3                                           | .6               | 10-20          | P                          |
| B |                  |                  |      | 60                                        | 30               | 10   | 930                 | 2.5                  | 96                                    | 6.4                                           | .5               | 10-20          | P                          |
| C |                  |                  |      | 54                                        | 26               | 20   | 930                 | 2.5                  | 98                                    | 6.2                                           | .5               | 10-20          | P                          |
| D |                  |                  |      | 44                                        | 21               | 35   | 930                 | 2.5                  | 98                                    | 5.8                                           | .4               | 10-20          | P                          |
| E |                  |                  |      | 40                                        | 20               | 40   | 930                 | 2.5                  | 98                                    | 7.2                                           | .4               | 10-20          | P                          |
| F |                  |                  |      | 24                                        | 11               | 65   | 930                 | 2.5                  | 98                                    | 403                                           | .4               | 10-20          | P                          |
| G |                  |                  |      | 62                                        | 33               | 5    | 900                 | 1.5                  | 95                                    | 6.0                                           | .6               | 10-20          | P                          |
| H |                  |                  |      | 60                                        | 30               | 10   | 900                 | 1.5                  | 95                                    | 5.4                                           | .4               | 20-15          | P                          |
| I |                  |                  |      | 54                                        | 26               | 20   | 900                 | 1.5                  | 96                                    | 7.1                                           | .4               | 10-15          | P                          |
| J |                  |                  |      | 44                                        | 21               | 35   | 900                 | 1.5                  | 98                                    | 4.3                                           | .4               | 10-15          | P                          |
| K |                  |                  |      | 40                                        | 20               | 40   | 900                 | 1.5                  | 98                                    | 5.0                                           | .3               | 10-15          | P                          |
| L |                  |                  |      | 24                                        | 11               | 65   | 900                 | 1.5                  | 98                                    | 6.6                                           | .3               | 10-15          | P                          |
| M |                  |                  |      | 62                                        | 33               | 5    | 950                 | 2.0                  | 98                                    | 4.9                                           | .5               | 10-20          | P                          |
| N |                  |                  |      | 60                                        | 30               | 10   | 950                 | 2.0                  | 98                                    | 5.9                                           | .6               | 10-20          | P                          |
| O |                  |                  |      | 54                                        | 26               | 20   | 950                 | 2.0                  | 98                                    | 6.2                                           | .7               | 10-20          | P                          |
| P |                  |                  |      | 44                                        | 21               | 35   | 950                 | 2.0                  | 98                                    | 6.7                                           | .8               | 10-20          | P                          |
| Q |                  |                  |      | 800                                       | 1                |      |                     |                      | 50                                    | 4.1                                           | .01-0.1          | 1-2            | C                          |
| S |                  |                  |      | 875                                       | 6                |      |                     |                      | 99                                    | 4.2                                           | .07-15           | 1-5            | P                          |
| T |                  |                  |      | 925                                       | 0.5              |      |                     |                      | 90                                    | 4.9                                           | 0.3-5            | 5-15           | P                          |
| U |                  |                  |      | 925                                       | 1.0              |      |                     |                      | 95                                    | 7.2                                           | 0.2-5            | 5-20           | P                          |
| V |                  |                  |      | 925                                       | 2.5              |      |                     |                      | 98                                    | 6.3                                           | 0.1-5            | 10-20          | P                          |
| W |                  |                  |      | 925                                       | 5.0              |      |                     |                      | 99                                    | 7.9                                           | 0.3-5            | 15-30          | P                          |
| X |                  |                  |      | 925                                       | 7.5              |      |                     |                      | 99                                    | 8.8                                           | 0.2-6            | 20-40          | P                          |
| Y |                  |                  |      | 1,025                                     | 1.0              |      |                     |                      | 95                                    | 5.6                                           | 1-2              | 50-100         | I                          |
| Z |                  |                  |      | 1,025                                     | 2.5              |      |                     |                      | 99                                    | 6.2                                           | 1-3              | 75-150         | I                          |

<sup>1</sup> C = Colloidal; P = Pigmentary; I = Insulating.

runs are shown in runs A through K of (b) in Table V below.

TABLE V  
(a) Preparation of Sodium Titanate Fibers

|     | Ingredients      |                  |      | Composition of Reaction Mix, Parts by Wt. |                  |      | Temp., °C. | Time, Hrs. | Conversion to Fibers of Size, Percent | Analysis of water Extracted Product, Mole Ratio TiO <sub>2</sub> /M <sub>2</sub> O | Size Category <sup>1</sup> |
|-----|------------------|------------------|------|-------------------------------------------|------------------|------|------------|------------|---------------------------------------|------------------------------------------------------------------------------------|----------------------------|
|     | TiO <sub>2</sub> | M <sub>2</sub> O | Salt | TiO <sub>2</sub>                          | M <sub>2</sub> O | Salt |            |            |                                       |                                                                                    |                            |
| A   |                  |                  |      |                                           |                  |      | 850        | 1          | 100                                   | 4.3                                                                                | C                          |
| B   |                  |                  |      |                                           |                  |      | 850        | 3          | 100                                   | 4.9                                                                                | C                          |
| E   |                  |                  |      |                                           |                  |      | 925        | 0.5        | 50                                    | 5.8                                                                                | P                          |
| F   |                  |                  |      |                                           |                  |      | 925        | 1.5        | 70                                    | 7.9                                                                                | P                          |
| G   |                  |                  |      |                                           |                  |      | 925        | 3.5        | 95                                    | 4.9                                                                                | P                          |
| H   |                  |                  |      |                                           |                  |      | 975        | 0.5        | 60                                    | 5.8                                                                                | P                          |
| I   |                  |                  |      |                                           |                  |      | 975        | 2.0        | 80                                    | 5.7                                                                                | P                          |
| J   |                  |                  |      |                                           |                  |      | 975        | 3.5        | 95                                    | 5.9                                                                                | P                          |
| K   |                  |                  |      |                                           |                  |      | 1,025      | 0.5        | 70                                    | 6.1                                                                                | I                          |
| L   |                  |                  |      |                                           |                  |      | 1,025      | 1.0        | 80                                    | 7.3                                                                                | I                          |
| M   |                  |                  |      |                                           |                  |      | 1,025      | 2.0        | 90                                    | 6.4                                                                                | I                          |
| N   |                  |                  |      |                                           |                  |      | 1,025      | 3.0        | 95                                    | 7.9                                                                                | I                          |
| O   |                  |                  |      |                                           |                  |      | 1,100      | 1.0        | 80                                    | 5.9                                                                                | I                          |
| P   |                  |                  |      |                                           |                  |      | 1,100      | 2.5        | 90                                    | 5.8                                                                                | I                          |
| Q   |                  |                  |      |                                           |                  |      | 1,150      | 5.0        | 99                                    | 6.6                                                                                | I                          |
| S   |                  |                  |      |                                           |                  |      | 1,050      | 2.5        | 96                                    | 6.3                                                                                | I                          |
| U   |                  |                  |      |                                           |                  |      | 950        | 2.5        | 95                                    | 5.2                                                                                | P                          |
| V   |                  |                  |      |                                           |                  |      | 1,050      | 4.0        | 98                                    | 6.7                                                                                | P                          |
| W   |                  |                  |      |                                           |                  |      | 900        | 2.0        | 98                                    | 5.7                                                                                | I                          |
| X   |                  |                  |      |                                           |                  |      | 975        | 2.5        | 98                                    | 5.8                                                                                | P                          |
| Y   |                  |                  |      |                                           |                  |      | 975        | 3.0        | 98                                    | 6.3                                                                                | P                          |
| Z   |                  |                  |      |                                           |                  |      | 975        | 4.0        | 98                                    | 7.1                                                                                | P                          |
| A-1 |                  |                  |      |                                           |                  |      | 1,025      | 1.0        | 98                                    | 6.2                                                                                | P                          |
| B-1 |                  |                  |      |                                           |                  |      | 1,025      | 2.5        | 99                                    | 6.2                                                                                | P                          |

## (b) Preparation of Mixed Na-K Titanate Fibers

| Ingredients        |                    |      | Composition of Reaction Mix, Parts by Wt. |                  |      | Temp., °C. | Time, Hrs. | Conversion to Fibers of Size, Percent | Analysis of Product                            |                     |                      | Size Category <sup>1</sup> |
|--------------------|--------------------|------|-------------------------------------------|------------------|------|------------|------------|---------------------------------------|------------------------------------------------|---------------------|----------------------|----------------------------|
| TiO <sub>2</sub>   | M <sub>2</sub> O   | Salt | TiO <sub>2</sub>                          | M <sub>2</sub> O | Salt |            |            |                                       | Mole Ratio TiO <sub>2</sub> /M <sub>2</sub> O  | Diam. avg., Microns | Length avg., Microns |                            |
| A- Rutile pigment  | NaHCO <sub>3</sub> | KCl  | 1.5                                       | 1                | 2.5  | 800        | 2          | 60                                    | 6/1.5 Na <sub>2</sub> O-0.5 K <sub>2</sub> O-- | 0.008               | 2.6                  | C                          |
| B- Rutile pigment  | NaHCO <sub>3</sub> | KCl  | 1.5                                       | 1                | 2.5  | 925        | 2.5        | 88                                    | 6/1.1 Na <sub>2</sub> O-0.8 K <sub>2</sub> O-- | 0.3                 | 35                   | P                          |
| C- Rutile pigment  | NaHCO <sub>3</sub> | KCl  | 1.5                                       | 1                | 2.5  | 1,070      | 4.0        | 95                                    | 6/1.0 Na <sub>2</sub> O-0.7 K <sub>2</sub> O-- | 1.1                 | 110                  | I                          |
| D- Anatase pigment | NaOH               | KCl  | 3                                         | 1                | 1.5  | 1,025      | 3          | 91                                    | 5.8/1.0 Na <sub>2</sub> O-1 K <sub>2</sub> O-- | 0.85                | 99                   | I                          |
| E- Anatase pigment | KOH                | NaF  | 2.5                                       | 1                | 2.5  | 1,075      | 3          | 96                                    | 4.3/1 Na <sub>2</sub> O-1 K <sub>2</sub> O--   | 0.90                | 130                  | I                          |
| L- Rutile ore      | Na <sub>2</sub> O  | KCl  | 70                                        | 23               | 7    | 850        | 3          | 92                                    |                                                |                     |                      | C                          |

<sup>1</sup> C=Colloidal; P=Pigmentary; I=Insulating.

## Example VI

Fibrous potassium titanate pigment was prepared by dissolving eleven parts of solid KOH pellets (83% KOH) or an amount of KOH equivalent to 9.2 parts (0.160 moles) in 5 mls. of water in a vessel to form a clear solution. 20 parts (0.25 mole) of TiO<sub>2</sub> (TiO<sub>2</sub>/K<sub>2</sub>O=3/1) and 9 parts of KCl (24% KCl in dry mix) were added to the solution with sufficient stirring to form a smooth paste which was placed in an oven at 150° C. and heated to dryness. The dry lump product recovered was then ground to pass a 30 mesh screen and the pulverized product was placed in a crucible and calcined at 945° C. for 70 minutes. Upon cooling, the mass was broken up into small lumps and soaked for two days in deionized water. Afterward, the lumps were leached free of KCl and excess KOH in a counter current flow of hot water and steam until the mole ratio of TiO<sub>2</sub>/K<sub>2</sub>O was determined to be 6 by analyses.

The recovered fibrous material was then separated into individual fibers by passing a 10% fiber-deionized water suspension through a colloid mill three times. The 10% fiber mix was diluted to 15 gm./liter by adding further amounts of deionized water and was stirred. Heavier non-exfoliated material was allowed to settle out for 15 minutes and was separated from the lighter dispersed fibers by decantation. Sediment from this process was diluted to a 10% mixture again and passed through the colloid mill until complete dispersion was obtained when rediluted to 15 gm./liter.

The resulting dispersed fiber slurry was adjusted to a pH of 7.3 by adding sufficient dilute HCl and the fibers water flocculated by adding 5 mls. of 0.1 M MgSO<sub>4</sub> water solution and filtered off. The pad of fibers collecting on the filter was then washed with three separate 1 liter portions of deionized water to remove the flocculating agents. The 26 parts of recovered fibers was dried in an oven at 100° C., cooled and passed through a 12 mesh screen to produce a 57% yield of free flowing pigment useful in papermaking. When so employed, it was found to be easily dispersed in the beater.

Microscopic examination of the pigmenting fibers revealed that they averaged 5 to 50 microns in length and had a 0.1 to 0.6 micron diameter, with most being 0.3 micron in diameter.

## Example VII

Sodium titanate pigment fibers are prepared in substantially the same manner as described in Example VI. Twenty parts of TiO<sub>2</sub> (0.25 mole) contained in 60 parts of wet raw anatase TiO<sub>2</sub> from a sulfate hydrolysis process for precipitating the TiO<sub>2</sub> were mixed with 6.4 parts of NaOH pellets (0.16 mole) and 30 parts of NaCl and the resulting mixture was calcined at 940° C. for 75 minutes. Following flocculation and processing as in Example VI, the length of the fibers was found to be shorter than the potassium titanate fibers obtained in that example. That is, they were about 15 to 20 microns long, and had diameters of the order of 0.2 to 0.6 micron. When processed in papermaking, this product was found to be practically no different in performance over a pure TiO<sub>2</sub>.

pigment prepared from the conventional hydrolysis of a titania sulfate solution pure TiO<sub>2</sub> and that from the rutile ore.

## Example VIII

A mixture containing 600 parts of potassium carbonate, 1,200 parts of titanium dioxide, 600 parts of potassium chloride, the mole ratio of TiO<sub>2</sub>/K<sub>2</sub>O being 2.9/1 in the presence of 25 weight percent KCl, was dry mixed for 4.5 days in a drum roller. This material was then pressed into cylindrical briquettes approximately 3/4" x 1" in size which were continuously fed at a 30 to 40 lb./hour rate into a rotary calciner of the type described in the foregoing examples. The bed temperature of the kiln has a profile of 750±25° C. at the feed entrance and 910±25° C. at pigment exit, with a continuous gradient of temperature over the apparatus length. Residence time in the kiln was regulated to 2.5 to 3.5 hours by adjusting the pitch and rotary speed of the kiln and to provide about 1 to 2 hours calcination of the reaction mass at temperatures of from 875° C. to 975° C. Uniform bed depth was maintained within the kiln with a holdup amounting to 200 to 300 lbs. of feed material. A total of 1830 parts of briquettes containing the fibrous pigment were collected at the hot end of the kiln over a period of 69 hours. (The deficiency was due to about 250-300 lbs. of KCl which boiled out the feed port, loss of about 17 pounds of CO<sub>2</sub> from the reaction and kiln holdup.) The briquettes were then placed in a 1000 gal tank and leached with 90° C. demineralized water flowing at 3 gals./hr. for 6 days. The water was continuously changed until the leachings were free of chlorine and the leachable caustic was removed from the fibers. The recovered fibrous titanate, in the shape of briquettes, were placed on trays, and dried in an oven at 110° C.

Exfoliation of the dry fibers was performed by first dry grinding them to pass through a 4 mesh screen and then mixing them with demineralized water to form a 10% fiber slurry. This slurry was then passed through a conventional attrition mill set at 3 mils followed by dilution of the slurry to a 1.5% fiber content with additional demineralized water. This mixture was then passed through a cleaner apparatus consisting essentially of a wet cyclone separator to remove large particles of grit. Finally, the degritted slurry was reprocessed back through the attrition mill and the dispersion was allowed to settle for 2 hours. The top 10% of this liquid (300 gals.) containing the dispersed fiber was decanted and transferred to another vessel and processed in 300 gal. portions as follows: The dispersed fiber slurry was neutralized to a pH of 7.25 with 25% hydrochloric acid, then flocculated by adding 7 lbs. of KCl. Flocculated fibers were filtered on paper to form cakes 26" x 26" x 1" and were washed free of chloride with 3 portions of water, 9 gallons each. The filter cakes were placed on trays and dried at 75° C. for 24 hours. Moisture in the cake after drying averaged 3 to 5%. Dry filter cakes were exfoliated again by dry grinding to pass a 4 mesh screen, then micropulverized. A total of 1,150 pounds of fibers (80% yield) were collected. The bulk density of the finished pigment was 5 lbs./cu. ft.

## 11

and the fiber lengths varied between 10-40 microns with the average diameters of the product being 0.3 micron. 1000 pounds of this product was conventionally processed into a high quality magazine paper print of 70# ream weight wherein it proved to impart and provide better papermaking properties over a corresponding paper pigmented with  $TiO_2$ . This was especially true in respect to offset lithography performance. In addition, the treated paper embossed much easier, with much less pressure being required.

Compared to the  $TiO_2$  treated paper, the fibrous titanate-treated paper product was outstanding in brightness and less abrasive. In off-set printing, less slitter dusting was noted, the ink drying more rapidly, while the print definition was highly satisfactory. Its decreased abrasion property is especially advantageous in that the life of the Fourdrinier wire becomes extended, and cutter blade wear and dusting on the sheet during cutting is decreased, as is printing press plate wear.

## Example IX

A paste containing 1000 parts  $TiO_2$ ; 500 parts  $K_2CO_3$ ; 200 parts  $K_2SO_4$ ; 700 parts KCl and 1,875 parts  $H_2O$ , was dried at 120° C. in a tray dryer and then briquetted into 1" x 3/4" squares. The mole ratio of  $TiO_2/K_2O$  in the dry mix was 2.7/1 in the presence of 30% KCl. The briquettes, with a bulk density of 70 lbs./cu. ft., were fed into a 10 in. diameter by 15 ft. ceramic lined shaft furnace to a depth of 8-11 ft. The rate of feeding was so regulated that residence time in the kiln was about 8 hours. The furnace was direct fired with a natural gas-air mixture such that the hot combustion gases passed up through the bed to provide a countercurrent flow of hot combustion products over the briquette bed. Calcined fibrous product was removed from the bottom of the furnace by periodically opening its outlet grates. After about 6 hours of feed to a bed which started at a depth of four feet, the temperature profile is about 975° C. at the bottom and 750° C. at the top. At the end of such 6 hours of feed, the rate of movement through the furnace was controlled at one foot/hr. so that the residence time at 875° C. to 950° C. was about 1.5 to 3.5 hours and held within that average rate for 60 hours. These temperatures were maintained by adjusting the gas flame used to directly fire the furnace and by adjusting the throughput rate. About 2050 parts of calcined material was produced.

Briquettes containing the fibrous pigment product were processed in a 1000 gal. tank, exfoliated and dried as outlined in Example VIII. A total of 1100 lbs. of exfoliated fibers (91% yield) was obtained. The bulk density of the finished pigment averaged 5.1 lbs./cu. ft., its fiber lengths varied from 15-50 microns, and its diameters ranged from 0.09 to 0.31 micron, 600 lbs. of the product was incorporated into 40# ream weight magazine print to provide a paper having superior brightness, slitter dusting, print definition and embossing characteristics.

## Example X

A mixture containing 424 parts of sodium carbonate, 1100 parts  $TiO_2$ , 200 parts of sodium chloride, the mole ratio of  $TiO_2/Na_2O$  being 6/2 in the presence of 1700 parts of NaCl (52% of the mix) were blended for 3 days in a drum roller. The resulting mixture was then briquetted and calcined in a rotary kiln as described in Example VIII. The feed rate and flame temperature were regulated to hold the residence time of 1 to 2 hours at 900° C  $\pm 25^\circ$  C. About 1200 lbs. of fibrous sodium hexatitanate material was obtained after leaching and exfoliating in accordance with the procedure outlined in Example VIII. The fibers averaged 0.67 micron in diameter with lengths up to 50 microns. These sodium hexatitanate fibers were found to be slightly softer and more flexible than the above potassium fibers. When incorporated into paper, these pigmentary fibers possessed brightness slightly su-

erior to that obtained from fibrous potassium titanate pigment use.

## Example XI

A mixture of 160 parts NaOH, 280 parts  $K_2CO_3$ , 1250 parts  $TiO_2$  in ground rutile ore, 175 parts NaCl, and 175 parts KCl were dry blended in a drum roller for a period of 3.5 days. The mole ratio of  $TiO_2/M_2O$  was 3.9/1, in the presence of 17% alkali chlorides. This material was briquetted and processed in a direct fired rotary kiln as described in Example VIII.

Approximately 1050 lbs. of fibrous pigment was recovered after leaching and exfoliation as set forth in said example. On analysis, the fibers were found to have the general composition  $Na_{0.8}K_{1.2}Ti_6O_{13}$ . When incorporated into a paper, they performed equally as well as the pure potassium hexatitanate pigments of this invention in papermaking.

## Example XII

20 A pulp beater was charged with 445 parts of 4% sulfite pulp-water slurry containing 18 parts of sulfite pulp then with 7,000 mls. of distilled water and stirred for 4 minutes. To this was added 1.88 parts of fibrous potassium hexatitanate pigment having an average diameter of 0.3 25 micron and lengths ranging between 40 and 150 microns, and an additional 4 minutes of stirring was undertaken. 1.78 parts of 20% starch solution and 17.8 mls. of 4% alum was then added with 4 minutes of stirring being applied for each ingredient.

30 The resulting slurry was placed into a proportionator and diluted to 12,600 mls. with distilled water, and thirteen 8" x 8" sheets of paper were then sheeted on a 100 mesh screen in a conventional type sheeting machine by withdrawing 970 mls. for each sheet. The dry weight 35 for each sheet averaged 1.45 parts, equivalent to 25 lb. ream weight. Opacity, brightness and retention characteristics of these sheets were measured. The average of these sheets for various loadings is recorded in the following table:

TABLE VI

| 45 | Loading, Weight Percent |                            | Paper Properties                       |                 |          |
|----|-------------------------|----------------------------|----------------------------------------|-----------------|----------|
|    | Percent $TiO_2$         | Percent Potassium Titanate | Percent Retained $TiO_2$ Plus Titanate | Percent Opacity |          |
|    |                         |                            |                                        | Waxed           | Nonwaxed |
| 50 | 10                      | -----                      | 7.25                                   | 25              | 61.1     |
|    | -----                   | 2.5                        | 29.0                                   | 19.1            | 59.8     |
|    | -----                   | 5                          | 31.3                                   | 25.2            | 64.0     |
|    | -----                   | 10                         | 42.0                                   | 38.1            | 71.3     |

## Example XIII

55 Employing the procedures of Example XII for a 13 sheet evaluation procedure, the following results were obtained when mixtures of pigmentary fibrous potassium titanates of this invention were employed in conjunction with a commercial grade  $TiO_2$  pigment. The potassium titanate fibers used for this series were slightly longer than those employed in Example XII, i.e., their lengths were 50 to 300 microns and their diameter was about 0.25 micron:

TABLE VII

| 65 | Loading, Weight Percent |                            | Paper Properties                       |                 |          |
|----|-------------------------|----------------------------|----------------------------------------|-----------------|----------|
|    | Percent $TiO_2$         | Percent Potassium Titanate | Percent Retained $TiO_2$ Plus Titanate | Percent Opacity |          |
|    |                         |                            |                                        | Waxed           | Nonwaxed |
| 70 | 10                      | 0                          | 9.6                                    | 27.9            | 57.7     |
|    | 8                       | 2                          | 17.9                                   | 28.6            | 59.2     |
|    | 6                       | 4                          | 31.5                                   | 31.5            | 61.4     |
|    | 0                       | 10                         | 42.0                                   | 38.1            | 71.3     |

**13**  
*Example XIV*

A series of 25 lb. and 50 lb. ream weight sheets filled with a fibrous potassium hexatitanate pigment 16 to 40 microns in length and having an average 0.25 micron diameter, were prepared for comparison with similarly prepared and weighted sheets filled with anatase  $TiO_2$  pigment. The following are the comparative results:

TABLE VIII.—25 POUND REAM WT. SHEETS

| Pigment                 | Percent Pigment Addition | Percent Opacity Nonwaxed | Waxed | Percent Pigment Retention | Bursting Strength |
|-------------------------|--------------------------|--------------------------|-------|---------------------------|-------------------|
| Sulfite Pulp-----       | 0                        | 53.7                     | 12    | 0                         |                   |
| $TiO_2$ -----           | 10                       | 58.7                     | 24.2  | 9.2                       |                   |
| $TiO_2$ -----           | 20                       | 59.8                     | 26.7  | 7.7                       |                   |
| Potassium Titanate----- | 5                        | 59.7                     | 21.2  | 20.0                      |                   |
| Do-----                 | 10                       | 63.4                     | 28.8  | 23.1                      |                   |
| Do-----                 | 20                       | 69.6                     | 38.7  | 21.0                      |                   |

50 POUND REAM WT. SHEETS

|                         |    |      |      |      |      |
|-------------------------|----|------|------|------|------|
| Sulfite Pulp-----       | 0  | 72.5 | 15.3 | 0    | 26.2 |
| $TiO_2$ -----           | 5  | 74.0 | 25.5 | 6.8  | 26.3 |
| $TiO_2$ -----           | 10 | 75.2 | 30.5 | 6.8  | 25.4 |
| $TiO_2$ -----           | 20 | 76.8 | 36.9 | 8.3  | 25.3 |
| Potassium Titanate----- | 5  | 77.0 | 32.4 | 20.0 | 25.5 |
| Do-----                 | 10 | 80.3 | 43.9 | 23.1 | 24.7 |
| Do-----                 | 20 | 85.5 | 53.1 | 24.5 | 20.4 |

From this table it will be noted that opacity is improved significantly for papers of both ream weights without any significant decrease in bursting strength at the 5-20% retention level. The bursting strength values given in this and subsequent examples were determined in accordance with the Mullen method described in Technical Association of the Pulp and Paper Industry (TAPPI) #T-403.

*Example XV*

Following the procedure outlined in Example XII, a series of 25 lbs. ream wt. hand sheets were prepared, using fibrous sodium hexatitanate in the unleached crude

30 resulting paper to provide the results shown in Table X below.

In preparing the sheets, sulfite pulp was beaten in a conventional papermaker beater to a degree of 32° at a stock consistency of 4%. Fibrous potassium titanate pigment having a 10 to 45 micron length and average diameter of 0.275 micron or an anatase  $TiO_2$  pigment in the amounts specified in said table, were then added with the pulp which was then diluted and pumped to the headbox of the Fourdrinier machine. The pigmented-pulp slurry was then flocculated with alum in the headbox, with 2% alum on the O.D. pulp weight being used throughout. In no case was starch or rosin size used.

TABLE X

| Pigment                                      | Anatase— $TiO_2$ |       |       |      | Potassium Titanate Fibers |       |       |      | Pulp Only |
|----------------------------------------------|------------------|-------|-------|------|---------------------------|-------|-------|------|-----------|
|                                              | 5                | 10    | 15    | 20   | 5                         | 10    | 15    | 20   |           |
| Pigment Added, percent <sup>1</sup> -----    | 5                | 10    | 15    | 20   | 5                         | 10    | 15    | 20   | 0         |
| Pigment Analyzed, percent-----               | 7.07             | 10.49 | 13.59 | 4.44 | 8.92                      | 12.54 | 15.59 | 0    | 0         |
| Pigment in Dry Sheet (percent)-----          | 2.9              | 3.3   | 5.8   | 6.3  | 3.0                       | 6.8   | 8.8   | 12.4 | 0         |
| Pigment Retention (percent)-----             | 46.5             | 55.0  | 46.7  | 68.4 | 75.9                      | 69.5  | 79.7  | 0    | 0         |
| Dry Opacity (percent)-----                   | 84.0             | 84.1  | 87.4  | 88.9 | 85.4                      | 90.8  | 93.2  | 94.7 | 75.1      |
| Wax Opacity (percent)-----                   | 57.5             | 58.4  | 65.6  | 67.0 | 51.7                      | 62.8  | 67.9  | 72.1 | 22.6      |
| Brightness G.E. (percent)-----               | 83.4             | 86.3  | 87.0  | 87.3 | 84.3                      | 87.9  | 88.5  | 89.3 | 79.6      |
| Mullen Bursting Strength (lbs./sq. in.)----- | 24.0             | 26.6  | 23.4  | 21.3 | 22.7                      | 15.8  | 10.2  | 8.5  | 27.4      |
| Tear Strength:                               |                  |       |       |      |                           |       |       |      |           |
| Along-----                                   | 47               | 52    | 47    | 42   | 39                        | 42    | 44    | 48   | 50        |
| Across-----                                  | 68               | 63    | 64    | 49   | 53                        | 53    | 70    | 51   | 68        |

<sup>1</sup> Added on dry pulp basis.

<sup>2</sup> Analysis on dry pulp slurry.

kiln discharge as the pigmenting ingredient. This material averaged 25 microns in length and had an average diameter of 0.21 micron. The test results obtained in this series are shown in the following table.

The fibrous, water-insoluble alkali metal products of this invention in their colloidal, pigmentary or insulating form, vary in crystal structure depending on their history. The structure is that of the tetratitanate, hexatitanate or

TABLE IX

| Pigment              | Percent Pigment Addition | Percent Opacity Nonwaxed | Waxed | Percent Pigment Retention | Bursting Strength |
|----------------------|--------------------------|--------------------------|-------|---------------------------|-------------------|
| Sodium Titanate----- | 5                        | 58.9                     | 20.1  | 20.5                      | 16                |
| Do-----              | 10                       | 61.1                     | 26.3  | 22.6                      | 15.3              |
| Do-----              | 15                       | 63.5                     | 29.2  | 23.2                      | 14.2              |
| Do-----              | 20                       | 67.2                     | 37.4  | 25.3                      | 13.1              |

mixtures of both. They differ only in respect to size—that is fibrous products with diameters ranging from 0.005–0.1 micron and lengths at least 10 times the diameter are of colloidal size; those having diameters ranging from 0.1–0.6 micron and lengths ranging from 10 to 100 times their diameter are of pigmentary size; while products possessing diameters ranging from 0.6–3.0 microns and lengths ranging from 100 to 1000 times their diameter are of insulating or reinforcing type.

Essentially the invention entails an improved method for the selective preparation through selective control over the reactants and reaction conditions in a kiln process, of good yields on a continuous industrial basis, of predominantly (above 50% and preferably at least 80% or 90%) amounts of a fibrous colloidal, pigmentary or insulating titanate product. Although generally applicable to the preparation of alkali metal titanates, the process is especially useful for producing the preferred fibrous sodium and potassium titanates. Again, while described as applied to certain specific embodiments involving particular kiln calcinations, reactants, ratios, temperatures, times, etc., variance therefrom is contemplated. In general, any basic, water-soluble, oxygen-containing compound of an alkali metal oxide or salt which exists as the alkali metal oxide under reaction conditions (potassium, sodium, cesium, rubidium) e.g. an oxide, hydroxide, carbonate, bicarbonate, oxalate, nitrate, etc. or mixtures of such compounds can be used. Specific examples of such compounds include:  $\text{Na}_2\text{O}$ ,  $\text{NaOH}$ ,  $\text{NaNO}_3$ ,  $\text{Na}_2\text{CO}_3$ ,  $\text{NaHCO}_3$ ,  $\text{Na}_2\text{C}_2\text{O}_4$ ,  $\text{K}_2\text{O}$ ,  $\text{KOH}$ ,  $\text{K}_2\text{CO}_3$ ,  $\text{KNO}_3$ ,  $\text{KHCO}_3$ ,  $\text{K}_2\text{C}_2\text{O}_4$ ,  $\text{CsNO}_3$ ,  $\text{Cs}_2\text{O}$ ,  $\text{CsOH}$ ,  $\text{Cs}_2\text{CO}_3$ ,  $\text{CsHCO}_3$ ,  $\text{Cs}_2\text{C}_2\text{O}_4$ ,  $\text{Rb}_2\text{O}$ ,  $\text{RbNO}_3$ ,  $\text{RbOH}$ ,  $\text{Rb}_2\text{CO}_3$ ,  $\text{RbHCO}_3$ ,  $\text{Rb}_2\text{C}_2\text{O}_4$ ,  $\text{RbHSO}_4$ , and the like.

While  $\text{TiO}_2$  (titania) in either anatase or rutile anhydrous pigmentary or hydrated (orthotitanic acid) form comprises a preferred source of titanium for use in the invention, other titanium-oxygen compounds adapted to yield  $\text{Ti}_2$  under the reaction conditions can be employed. Examples thereof include the various sodium or potassium salts of titanic acid, e.g. meta or ortho titanates ( $\text{M}_2\text{TiO}_3$  or  $\text{M}_4\text{TiO}_4$ ), titanium hydroxide, titanyl sulfate ( $\text{TiOSO}_4$ ) or titanyl chloride. Similarly useful are certain types of titaniferous ores, such as rutile, ilmenite or beneficiated ilmenite, etc.

The source of titanium dioxide is probably the most dependent ingredient variable in the process. The size of the fiber and its rate of growth will depend upon the crystalline form of the  $\text{TiO}_2$ , its particle size, history and impurity content. Within any given source of titanium dioxide, an ore for example, the particle size of the ore will also affect the fiber growth characteristics. The degree to which the ore is ground prior to its compounding with the salt if present and the alkali metal oxide source will bear importantly on the preparation of a suitable fiber of particular size range. This is also true in preparing the fiber from hydrated titania or titanium dioxide pigment sources. Generally, finely ground (passing 325 mesh) titanium dioxide sources yield a higher degree of small particle size fiber and require higher temperatures to form materials of long fibrous nature. Coarse sources of titanium dioxide such as rutile (passing 60 mesh) yield fibers of intermediate range in predominantly pigmentary size. In explanation of this phenomena, it has been postulated that the formation of pigmentary fibers is a two step mechanism. In the first step, titanium dioxide is solvated in the salt matrix and reacts with the alkali metal oxide source to form an insoluble or rather less soluble fiber. These small fibers then at higher temperatures are redissolved and are recrystallized on the surface of larger fibers. It appears, therefore, that in very finely ground titanium dioxide or hydrated titania sources a predominance of colloidal material is formed rapidly, and that formation of larger fibers from this colloidal material is a slower process than large fiber formation directly from a relatively coarse  $\text{TiO}_2$  source.

On X-ray and chemical analysis, the products of this invention, depending on the temperature of calcination and the ratios of ingredients employed in their preparation, will be predominantly fibrous hexa- or tetratitanate in accordance with the formulae  $\text{M}_2\text{O}\cdot 6\text{TiO}_2$  or  $\text{M}_2\text{O}\cdot 4\text{TiO}_2$  wherein M is selected from the above enumerated alkali metals, and preferably, is sodium or potassium. An optimum type fibrous pigment or insulation composition is obtained by calcining pellets of well-blended  $\text{TiO}_2/\text{K}_2\text{CO}_3$ , in the molar ratio of 3/1 to 4/1 together with  $\text{KCl}$  (25–50% by weight total ingredients) at substantially 875–1050° C. temperatures. Thereafter the granular product is leached or water extracted and is then milled to effect separation of the fibers which are then collected and dried. As will be noted in such preparation recourse is had to an alkali metal halide, the presence of which provides a salt matrix or solvent in which the reaction can take place to grow fibers of the desired pigmentary or insulating size. The metal halide employed preferably consists of a chloride or fluoride of the same alkali metal as that of the oxide or its equivalent employed for reaction with the titanium-oxygen compound. Usually, alkali metal chloride concentrations of from 10% to 65% by weight of the total mix are effectively useful. In potassium titanate preparation the presence of from 10–30% potassium chloride is most satisfactorily useful while with sodium titanate preparation from about 30–75% of sodium chloride is needed. The ratio of  $\text{TiO}_2/\text{M}_2\text{O}$  can vary within the range mentioned above but preferably ranges from 6/1 to 6/3, with the best conversion to fiber being brought about when the indicated 3/1 to 4/1  $\text{TiO}_2/\text{K}_2\text{O}$  ratio of components is approximately maintained. If use is made of a dissimilar salt mixture, for example in the preparation of a sodium titanate with a fused potassium halide salt, the fibrous product will contain both sodium and potassium. Both alkali metal fluorides and chlorides with alkali metal chlorides being preferred for employment since they prove particularly suitable in the formation of fibers with a tetratitanate structure as well as the hexatitanate structure. The temperature required for the conversion in the presence of fluoride salts will be found to be somewhat lower than that necessary when chloride salts are present.

Generally, the higher the temperature the higher will be the solubility in the salt matrix of both the reactants and the fibers produced. About 5% to about 65% salt by weight is generally satisfactory for a continuous process wherein the fibers are being formed over a short time period. The quantity of salt needed in the reaction mix depends on two or three variables. The first variable is the degree to which the reactants are ground, the second variable is the temperature at which the operation is to be carried out, while the third variable is the type fiber being formed, either potassium or sodium titanate fiber. In forming sodium titanate, higher concentration (40–65% of the total mix) of salt is necessary for good fiber conversion, whereas in the case of potassium fiber formation anywhere from 5–40% proves suitable, depending upon temperature and the material desired as the end-product. Increasing the salt concentration in a particular reaction mix provides a more uniform product and the distribution of a particular particle size becomes less scattered. By this is meant that the scattering of oversized and undersized material is decreased to a point such that the product is more uniform in length and diameter than it is when lower concentrations of salt are used. At low concentrations of salt it has been found that fibers of the smaller dimension are predominant. This refining action appears to take place by redissolving the quickly formed smaller titanate fibers and their recrystallization on the surface of larger less soluble fibers. This refining action is particularly noticeable for fiber diameter, rather than fiber length. Nonacicular material is redissolved in the fused salt and then deposited on the surface of a larger fiber and renders the material, particularly in the inter-

mediate size ranges, free of very small fibers and non-acicular particles. Although the salt functions primarily as a flux in which the reaction takes place, it also to some unknown degree participates in the fiber formation and by a mechanism not clearly understood. When potassium titanate fibers are formed from titanium dioxide and potassium carbonate in, for example, a sodium salt, titanate fibers are obtained containing sodium in the lattice structure. Conversely, when sodium titanates are formed in the presence of potassium chloride one obtains potassium in the fiber structure. It will be understood that the presence or addition of relatively small amounts of various salts or impurities, including those of Mg, Al, Zn, and Ca, will affect the temperature of calcination required, the ingredient ratios used, the growth characteristics, and will generally alter the process of fiber formation. To compensate for these variances, use is contemplated of calcination temperatures substantially in excess of the range limits which have been indicated, particularly in those instances where production of pigmentary and insulating forms of titanate products is being undertaken.

Any known method for intimately mixing or blending the reactant ingredients prior to calcining them in dry, non-fluid form or compacted form can be resorted to. Higher density compacts afford better control of product fiber length and diameter and hence are preferred for use. These can be obtained in several ways. Thus a paste of the ingredients can be added to the kiln directly or evaporated on trays to form a solid mass which can then be broken into desirable sizes, or a dry mix of the powdered mixture can be pelletized or briquetted to suitable size through use of standard pelletizing and briquetting equipment and techniques to form the lumps or pellets to be fed to the kiln.

While the temperature of calcination is the dominant control variable in the process for forming a particular fibrous product, it may range generally from 800-1100°. However, as previously indicated, the fiber lengths are controlled primarily by the particular temperature at which the reaction mix is calcined. That is, use of the lower portion of such range, preferably from 600-850° C., provides fibers of predominantly colloidal size, while the temperature range from 875-975 provides predominantly intermediate or pigmentary size fibers; while temperatures ranging from 975-1050° C. results in the production of relatively long fibers, or predominantly insulation size material. These ranges apply to potassium titanate formation. When sodium titanate fiber formation is undertaken, temperatures ranging up to about 25° higher for each category are resorted to.

The temperature of calcination used for the production of a particular fiber is also dependent upon the source of titanium dioxide used in the reaction charge. Generally, the finer the titanium dioxide particles, the higher will be the temperature required; for example, a higher temperature is required for raw hydrous titania than for pigmentary  $TiO_2$ , which in turn requires a higher temperature than crude  $TiO_2$ , such as a titaniferous ore. The temperature of the salt matrix, when present, must be high enough to redissolve the small particle size fibers in order to recrystallize them on the surface of larger fibers already in formation. In finely divided mixes, formation of small fibers is relatively rapid and higher temperatures are therefore required for dedissolution. If a coarsely-ground titanium dioxide source is present, fiber formation is usually directed from the  $TiO_2$  source through the salt matrix and directly onto the fiber. Therefore, redissolution is not necessary. For this reason fiber formation usually takes place at a lower temperature.

The type of heating employed appears to have little effect upon the growth of a given fiber. Therefore, the type of furnacing or calcination means used is not important in comparing a shaft furnace with a rotary kiln, for example. Rather, it is the length of time to which the reactants are subjected to the prescribed temperature which is important.

The time and temperature needed for production of the desired fiber size is related to the  $TiO_2/M_2O$  mole ratio, the salt content (when present) and the size and density of the compacted feed charge. The fibers will be found to grow quite rapidly at first, usually within a half hour from commencement of the calcination. In extending the period of treatment at a given temperature, the fibers grow at the expense of smaller, previously formed fibers in the colloidal range. Their growth is just about linear with respect to time after a period of about 1 hour. The briquette or pellet size used is also a variable which effects the time at given temperatures, especially in a continuous process, such as that carried out in the rotary kiln where the pellet is heated gradually to the desired temperature. Radiant heat causes the temperature on the surface of the lump to rise faster than that within its interior and forms an envelope of small fibers around the pellet or briquette. These fibers, due to their ability to reflect radiation, tend to slow down heat penetration into such interior. It will be found desirable therefore to heat up slowly the entire compact to about 800° prior to elevating its temperature to the reaction temperature necessary for fiber and particle size formation. This can be effected by adjusting the speed at which the lumps are passing through the low temperature end of a direct fired rotary kiln or shaft furnace. This is particularly a factor in furnaces and continuous processes in which the heating is carried out by radiation, convection and conduction.

The fiber-containing reaction mixture obtained when a salt matrix is employed will be somewhat cemented together. It is then necessary to separate the fibers from the salt matrix and unreacted materials. In such instances, the procedures used for separating the fibers into various desired size ranges will differ in some aspects. In general, fiber separation from the reaction mixture is effected by leaching out the unreacted materials and the matrix salt in aqueous slightly acidic solution. On dissolving out the unreacted material and salt, the fibers are filtered and washed free of undesired materials with water prior to drying.

Colloidal size fibers can readily be separated in this manner by first grinding the kiln effluent into a pulverized mass and then by leaching the resulting material with water, using a high speed agitator, until unreacted materials present are dissolved. The aqueous blend, which is usually at a pH above 11, is then adjusted with a mineral acid or organic acid such as acetic acid to a pH of about 9-11. The resulting slurry is then passed 4-6 times through a colloid mill or other similar type mill until the fibers separate from coarse, unreacted particles which are emitted with the undispersed kiln effluent. The slurry-containing coarse material is then passed through a centrifuge or similar type separatory apparatus to remove said coarse particles from the colloidal suspension of fibers. The colloidal suspension, free of large coarse particles, must then be flocculated in such manner that the colloid can be filtered and dried without agglomeration or recementing of the fiber. This requires special handling techniques different from those applied to larger or insulating sized fibers. To effect such flocculation, the suspension is first acidified to a pH of 6.5 by the incorporation of sufficient organic or inorganic cation-active compound, preferably a commercial type cationic ion-exchange resin which will replace the alkali metal cations in solution with protons and enable removal of the cationic solution through filtering from the colloid dispersion. Other useful forms of commercially available cationic ion-exchange compositions are those of the nuclear-sulfonic type, phenolic-methylene-sulfonic type, sulfonated coal types and carboxylic types. Inorganic types including aluminum silicate, silicic acid, etc. Upon freeing the dispersion of cations, anion removal must be undertaken which can be readily brought about by incorporating in the dispersion a sufficient amount of a conventional type weakly or strongly basic anion-exchange compound, preferably a commercially available

anion-exchange resin essentially to replace anions present with hydroxyl groups and in such manner that the displaced anions can be removed through filtering treatment. Upon cation and anion removal, flocculation of the colloidal particles is effected and by adding a conventional type flocculating agent, such as alum, or other suitable flocculating agents in minute traces containing cations such as manganese, zinc, copper, etc. The flocculated material can then be collected in a basket centrifuge or other suitable filtration equipment and dried at about 100° C.

Kiln discharge containing larger pigmentary or insulation size fiber material can be quenched directly as it issues from the kiln or it can be cooled, ground and then added to demineralized water as illustrated in the examples for the purpose of leaching out the fused salt present. Except in processing colloidal fibers the use of deionized water is not a requirement. One satisfactory method of separation comprises placing the kiln discharge in large tanks purged with 90° C. deionized water. Fresh demineralized water is continuously supplied to the tanks and until the leachings are found to be essentially free of halides and caustic. Fibrous titanate bundles in the shape of briquettes or pellets of the original sizes that were added to the kiln are then placed on trays to be dried. Unlike the colloidal particles, exfoliation of the dry particles can be effected by passing the material into and grinding it in a colloid type mill. Such grinding can be undertaken in several different ways. In preparing pigmentary and insulating size fibers, some treatment is necessary to remove any undesired larger sized or smaller sized particles, lumps of foreign material or agglomerates which might adversely affect their usefulness, particularly in paper applications. The refining stages to which these fibrous materials are subjected can consist of many steps. Usually, these entail a first step of grinding the freshly-leached lumps to a size of about 4 mesh screen; mixing the ground lumps with water to form an approximate 10% slurry; and then passing this slurry into an attrition mill set at about 1-5 mils for further treatment. Thereafter, the resulting material is diluted with water to about 1% solids and is passed through conventional separators to remove undesired large particles of grit. This can be carried out on a continuous recycle basis until all material passes particular standards. Upon requisite particle size being attained, the material is allowed to stand in large decantation tanks prior to filtration and flocculation treatment. Obviously methods are selected to minimize mechanical damage to the fibers.

As exemplified in the examples, the pigmentary fibrous titanates of this invention are particularly useful as inorganic pigmenting ingredients in paper manufacture. In such applications they advantageously reduce costs and impart high, increased opacity and brightness characteristics to the paper without any appreciable decrease in bursting strength. In addition the resulting paper product exhibits improved printability characteristics, especially in offset printing applications. The fibrous pigment is adaptable to any type of papermaking procedure which generally involves mixing the pigment, starch and other desired paper ingredients with the pulp slurry and preferably after the pulp has been suitably beaten in accordance with usual papermaking practice. Since the pigmentary titanate fibers disperse easily in paper pulp and are not seriously affected by the dispersing action of starch, they will be found to provide much greater pigment retention in the sheet than it provided with  $TiO_2$  when starch is present. Thus, when the paper retention properties of the fibrous pigment are compared with a titanium dioxide pigment a 20% to 30% better retention will be found to obtain for the fibrous pigment product of this invention.

The improvements thus afforded by reason of such fibrous titanate pigment employment in papermaking will vary somewhat depending on the pulps used but generally enhancement in opacity and other desired paper characteristics will inherently result with the use of all pulps and

combinations. Following dispersion of the pigmenting titanate in the pulp, the pH of the slurry is adjusted to within the range 4.5 to 6.5, and preferably to about pH of 5, by adding a flocculating agent such as aluminum sulfate, a salt of sulfuric acid or sulfuric acid per se. The acidified slurry is then transferred to the head box of a conventional papermaking apparatus, e.g. a Fourdrinier or cylinder machine and is sheeted into paper.

Although titanates with  $TiO_2/M_2O$  stoichiometry of 5/1 to 8/1 are preferred for use in such applications, the tetratitanates of potassium and sodium as well as sodium and potassium hexatitanates or mixtures of such titanates are also advantageously useful. Potassium hexatitanate fibers within the average diameter from 0.1 to 0.4 micron with lengths of 5-100 microns afford retention and overall pigment properties and hence are especially useful. For optimum retention, dispersion and opacity, preferred diameter and length sizes for either sodium or potassium fibrous titanates comprise from 0.2 to 0.3 micron in diameter and lengths of from 10 to 50 microns.

Sufficient titanate pigment is added to constitute from about 0.5 to 30% of the pulp on a dry basis. Ash values of the paper, by virtue of the high pigment retention obtained, will range from about 20% to 65% or 80% of the pigment concentration in the slurry on a dry pulp basis.

The invention is not limited to the addition of the fibrous titanate in the beater or doping box. The pigment may also be incorporated in paper coatings and folding 30 boxboard during or after the drying step. In folding boxboard applications, the titanate pigment plus starch coatings crack less on bending than coatings made from  $TiO_2$  and starch.

The titanate fibers in preferred diameter range bend 35 easily to decrease the abrasive wear on the Fourdrinier screen. This decreased abrasion is attributed to the intrinsic softness of the fibers, the entrainment of the paper pulp, and the alignment of the fibers on the moving screen. Such reduced abrasion also reduces the wear on the 40 pnuches, slitter knives and trimmer blades which decreases slitter dust contamination of printing plates in the letter press and blankets in the off-set press.

A further improvement which the invention affords in papermaking, particularly when 10% and over of the 45 fibrous titanate pigment is present in the paper arises from the high melting point of the fibers. Because titanate fibers do not melt or disintegrate below 1150° C. and the thin interwoven fibers retain a structural network similar to cellulose paper, papers containing them advantageously 50 retain sheet form and legibility of printing or writing after burning and thereby afford a desired preservation of records.

Another feature of titanate pigment use in paper is the 55 retardation against paper ageing which they provide. Yellowing and ageing is considered to be due to acid attack on the cellulose fibers, generated by hydrolysis of alum coagulating agent employed in papermaking. Alkali metal titanates possess residual alkalinity which advantageously neutralizes and prevents the very slow undesired 60 acid attack on cellulose.

Advantageously, this invention affords improved methods for producing novel forms of colloidal, pigmentary or insulating grades of fibrous alkali metal titanates in desired, uniform and requisite fiber dimension. This is 65 achieved by a controlled, uniform heating, in essentially "dry" state, of the specified ratios of reactants in relatively small, preferably modular state, e.g. less than 2" and preferably less than 1/2" size, to insure uniform heating throughout the entire charge to the peak temperature requisite for heat soak.

We claim:

1. A method for producing fibrous, water-insoluble alkali metal titanates in predetermined diameter-to-length size containing a molar ratio of  $TiO_2/M_2O$  (M being an alkali metal) of from 4:1 to 9:1, comprising calcining and react-

ing under essentially dry, non-fluid conditions a previously dry-blended, nodular compacted mixture of sufficient basic, water-soluble oxygen-containing alkali metal compound selected from the group consisting of an oxide, hydroxide, salt, and mixtures thereof, with an oxygen-containing titanium compound yielding  $TiO_2$  in the reaction, employing in the process calcination temperatures ranging from 200-850° C. when producing a predominantly colloidal size titanate having particle dimensions ranging from 0.005-0.1 micron diameter and lengths at least 10 times said diameter; calcination temperatures ranging from 850-975° C. when producing a predominantly pigmentary size titanate having particle dimensions ranging from 0.1-0.6 micron in diameter and length 10-100 times said diameter; and calcination temperatures ranging from 975-1150° C. when producing a predominantly insulating size titanate having particle dimensions ranging from 0.6-3.0 microns in diameter and lengths from 100-1000 times said diameter, leaching the titanate reaction product from the calcination to remove undesired reaction products therefrom, and then filtering, exfoliating, drying and recovering the desired fibrous titanate product.

2. The process of claim 1 in which the basic oxygen-containing alkali metal compound is a potassium compound.

3. The process of claim 1 in which the basic oxygen-containing alkali metal compound is a sodium compound.

4. The process of claim 1 in which calcination temperatures ranging from 600-825° C. are used in the production of a predominantly colloidal size titanate.

5. The process of claim 1 in which the oxygen-containing titanium compound is mineral rutile.

6. The process of claim 1 in which the oxygen-containing titanium compound is  $TiO_2$ .

7. The process of claim 1 in which the compacted reaction mixture subjected to calcination additionally contains from 10 to 30% by weight of an alkali metal halide.

8. The process of claim 4 in which the basic oxygen-containing alkali metal compound is a potassium compound.

9. The process of claim 4 in which the basic oxygen-containing alkali metal compound is a sodium compound.

10. The process of claim 4 in which the compacted mixture being calcined contains a molar ratio of titanium compound to alkali metal compound, calculated as  $TiO_2/M_2O$ , ranging from 2:1 to 8:1.

11. The process of claim 1 in which the dry, compacted mixture subjected to calcination additionally contains about from 5-65%, by weight, of an alkali metal halide.

12. The process of claim 11 in which the basic oxygen-containing alkali metal compound is a sodium compound and the alkali metal halide is sodium halide.

13. The process of claim 11 in which the basic oxygen-containing alkali metal compound is a potassium compound and the alkali metal halide is a potassium halide.

14. The process of claim 11 in which the oxygen-containing titanium compound is mineral rutile.

15. A method for preparing a fibrous water-insoluble alkali metal titanate containing a molar ratio of  $TiO_2/M_2O$  (M being an alkali metal) of from 4:1 to 9:1 and in predetermined diameter-to-length size and predominantly colloidal with at least 50% of its particles ranging in size from 0.005-0.1 microns diameter with lengths at least ten times said diameter, comprising calcining under essentially dry-non-fluid reaction conditions a previously dry-blended, nodular, compacted mixture of (1)  $TiO_2$ , (2) a basic water-soluble oxygen compound of an alkali metal selected from the group consisting of an oxide, hydroxide, salt, and mixtures thereof, in a molar ratio of  $TiO_2$  to alkali metal oxygen compound of from 2:1 to 8:1, and (3) 5-45 parts by weight of an alkali metal chloride, effecting said calcination at temperatures ranging from 600-850° C. until conversion to the alkali metal titanate is obtained,

and then leaching, filtering, drying and recovering the resulting fibrous colloidal titanate.

16. A method for preparing a fibrous water-insoluble alkali metal titanate containing a molar ratio of  $TiO_2/M_2O$  (M being an alkali metal) of from 4:1 to 9:1 and in predetermined diameter-to-length ratio with at least 50% of the titanate particles in insulating size having dimensions ranging from 0.6-3.0 microns in diameter and lengths 100-1000 times said diameter, comprising calcining under essentially dry, non-fluid conditions and in the form of a compacted, nodular dry-blended reaction mixture, 20-80 parts by weight of  $TiO_2$ , 7-65 parts by weight of a basic water-soluble oxygen compound of an alkali metal selected from the group consisting of an oxide, salt and mixtures, and from 5-45 parts by weight of an alkali metal chloride, effecting said calcination at temperatures ranging from 975-1100° C. and until conversion to the desired titanate is obtained and thereafter leaching, filtering, exfoliating, drying and recovering the fibrous insulating form of titanate product.

17. A method for preparing fibrous water-insoluble potassium titanate useful in constructing insulating blocks, said titanate being in predetermined diameter and length size with at least 50% of its particles ranging in dimension from 0.6-3.0 microns in diameter and 100-1000 times

the diameter in length, comprising calcining under essentially dry, non-fluid conditions and at a temperature ranging from 975-1050° C. a compacted, nodular dry-blended reaction mixture consisting of 45-55% by weight of KCl, the remainder being  $TiO_2$  and an alkali metal compound selected from the group consisting of  $KHCO_3$ ,  $K_2CO_3$ , and KOH, employing in the mixture a molar ratio of  $TiO_2/K_2O$  of about 3:1, effecting said calcination until conversion to potassium titanate is obtained, quenching the resulting calcined reaction product in water, and then filtering, exfoliating, drying and recovering the fibrous pigmentary potassium titanate.

18. A method for producing fibrous water-insoluble potassium titanate useful as loose bulk insulating material, said titanate being in predetermined diameter and length size with at least 50% of its particles ranging in dimension from 0.6-3.0 microns in diameter and 100-1000 times said diameter in length, comprising calcining at a temperature ranging from 975-1075° C. under essentially dry, non-fluid conditions, a nodular compacted previously dry-blended reaction mixture consisting of 20-30%, by weight, of KCl, the remainder being  $TiO_2$  and an alkali metal compound selected from the group consisting of  $KHCO_3$ ,  $K_2CO_3$  and KOH, employing in the reaction mixture a molar ratio of  $TiO_2/K_2O$  of about 3.5:1, continuing said calcination until conversion to potassium titanate is obtained, quenching the resulting calcined reaction product in water, and then filtering, exfoliating, drying and recovering the fibrous pigmentary potassium titanate product.

19. A method for producing fibrous water-insoluble potassium titanate useful as a paper pigment, said titanate being in predetermined diameter and length size with at least 50% of its particles ranging in dimension from 0.1-0.6 micron in diameter and 10-100 times the diameter in length, comprising calcining under essentially dry, non-fluid conditions and at a temperature ranging from 850-975° C. a compacted pelletized dry-blended reaction mixture consisting of 20-30% by weight of KCl, the remainder being  $TiO_2$  and an alkali metal compound selected from the group consisting of  $KHCO_3$ ,  $K_2CO_3$ , and KOH, employing in the mixture a molar ratio of  $TiO_2/K_2O$  of about 3.5:1, continuing the calcination until conversion to the desired fibrous potassium titanate is attained, quenching the pelletized calcined reaction product in water, and then filtering, exfoliating, drying and recovering the pigmentary fibrous product.

20. A method for producing fibrous water-insoluble potassium titanate useful in boxboard paper, said titanate being in predetermined diameter and length size with at

least 50% of its particles ranging in dimension from 0.1-0.6 micron in diameter and 10-100 times the diameter in length, which comprises calcining under essentially dry, non-fluid conditions and at a temperature from 850-975° C., a compacted, previously dry-blended pelletized mixture consisting of 20-30% by weight of KCl, the remainder being  $TiO_2$  and an alkali metal compound selected from the group consisting of  $KHCO_3$ ,  $K_2CO_3$  and KOH, employing in the mixture a molar ratio of  $TiO_2$  to  $K_2O$  of about 4:1, continuing the calcination until conversion to said titanate is attained, quenching the resulting pelletized reaction product in water, and then filtering, exfoliating, drying and recovering the desired titanate product.

21. A method for producing fibrous water-insoluble potassium titanate, useful as insulating pigment said titanate being in predetermined diameter and length size with at least 50% of its particles ranging in dimension from 0.1-0.6 micron in diameter and 10-100 times the diameter in length, which comprises calcining at a temperature ranging from 975-1050° C. under essentially dry, non-fluid conditions, a compacted, nodular, previously dry-blended reaction mixture consisting of 5-30% by weight of KCl, the remainder being  $TiO_2$  and an alkali metal compound selected from the group consisting of  $KHCO_3$ ,  $K_2CO_3$ , and KOH, employing in said mixture a molar ratio of  $TiO_2$  to  $K_2O$  of about 4.5:1, quenching the resulting reaction product in water and then filtering, exfoliating, drying and recovering the desired pigmentary titanate fibers.

22. A process for preparing a fibrous water-insoluble potassium titanate in predominantly pigmentary size dimension with at least 50% of its particles ranging from 0.1-0.6 micron in diameter and at least 10-100 times the diameter in length which comprises, subjecting a compacted, previously dry-blended, pelletized reaction mixture containing, by weight, 50% titanium dioxide, 25% potassium chloride and 25% potassium carbonate to calcination under essentially dry-non-fluid conditions in a rotary calciner at temperatures ranging from 875-975° C.

until conversion to potassium titanate is effected, quenching the pelletized calciner reaction product through discharge in water and leaching said product free of chloride salts, separating the fibrous particles by subjecting a dilute slurry thereof to milling treatment and until said pigmentary size titanate fibers remain, flocculating and then filtering said dilute slurry and then drying and recovering the desired fibrous pigmentary potassium titanate.

23. A method for preparing fibrous water-insoluble alkali metal titanate containing a molar ratio of  $TiO_2/M_2O$  (M being an alkali metal) of from 4:1 to 9:1 in predetermined diameter-to-length ratio and predominantly pigmentary in size with at least 50% of its particles having dimensions ranging from 0.1-0.6 micron in diameter and lengths 10-100 times said diameter, comprising calcining, under essentially dry, non-fluid conditions and in the form of a nodular compacted, previously dry-blended mixture, (1)  $TiO_2$ , (2) a basic water-soluble oxygen compound of an alkali metal selected from the group consisting of an oxide, hydroxide, salt, and mixtures of said compounds, in a molar ratio of  $TiO_2$  to  $M_2O$  (M being an alkali metal) of from 2:1 to 8:1, and (3) 5-45 parts by weight of an alkali metal chloride, effecting said calcination at temperatures ranging from 850-975° C. until conversion to an alkali metal titanate is obtained, and then quenching, leaching, filtering, exfoliating, drying and recovering the resulting fibrous pigmentary product.

30

## References Cited

## UNITED STATES PATENTS

|           |        |              |           |
|-----------|--------|--------------|-----------|
| 2,833,620 | 5/1958 | Gier et al.  | 23-51     |
| 2,841,470 | 7/1958 | Berry        | 23-51     |
| 2,924,549 | 2/1960 | Klein et al. | 162-162   |
| 3,129,105 | 4/1964 | Berry et al. | 106-299 X |

OSCAR R. VERTIZ, Primary Examiner.

H. T. CARTER, Assistant Examiner.

40